

# United States Patent [19]

Kaneko et al.

[11] Patent Number: 4,639,415

[45] Date of Patent: Jan. 27, 1987

[54] SILVER HALIDE COLOR PHOTOGRAPHIC MATERIAL CONTAINING A MAGENTA COLOR IMAGE-FORMING COUPLER

[75] Inventors: Yutaka Kaneko, Sagamihara; Toshihiko Kimura, Hino; Kenji Kadokura, Hachioji, all of Japan

[73] Assignee: Konishiroku Photo Industry Co., Ltd., Japan

[21] Appl. No.: 776,442

[22] Filed: Sep. 16, 1985

[30] Foreign Application Priority Data

Sep. 17, 1984 [JP] Japan ..... 59-194494  
Feb. 18, 1985 [JP] Japan ..... 60-31297

[51] Int. Cl.<sup>4</sup> ..... G03C 1/06; G03C 1/08; G03C 7/26; G03C 7/32

[52] U.S. Cl. ..... 430/558; 430/505;

430/551; 430/613; 430/614

[58] Field of Search ..... 430/558, 551, 505, 613, 430/614

[56] References Cited

U.S. PATENT DOCUMENTS

3,565,631 2/1971 Oguchi et al. ..... 430/551  
3,725,067 4/1973 Bailey ..... 430/470  
3,837,857 9/1974 Abbott ..... 430/551 X  
4,366,231 12/1982 Mayer et al. ..... 430/551 X  
4,396,707 8/1983 Von König et al. ..... 430/551 X  
4,418,142 11/1983 Langen et al. ..... 430/551 X  
4,518,679 5/1985 Leppard et al. ..... 430/551 X  
4,518,688 5/1985 Leppard et al. ..... 430/551

FOREIGN PATENT DOCUMENTS

1252418 11/1971 United Kingdom .  
1334515 1/1973 United Kingdom .  
2135788 9/1984 United Kingdom .

Primary Examiner—John E. Kittle

Assistant Examiner—Mukund J. Shah  
Attorney, Agent, or Firm—Finnegan, Henderson, Farabow, Garrett & Dunner

[57]

## ABSTRACT

A silver halide color photographic material is disclosed which contains a magenta color image-forming coupler represented by the following formula (I) and a compound represented by the following formula (II):



wherein Z represents the group of nonmetallic atoms necessary for forming a nitrogen-containing heterocyclic ring, provided that the ring to be formed by said Z may have a substituent;

X represents a hydrogen atom or a substituent capable of leaving upon reaction with the oxidized product of a color developing agent; and

R represents a hydrogen atom or a substituent.



wherein R<sub>1</sub> is an aliphatic group, a cycloalkyl group or an aryl group; and

Y represents the group of nonmetallic atoms necessary for forming a 5- to 7-membered heterocyclic ring taken together with the nitrogen atom, provided that at least two hetero atoms among the heterocyclic ring-forming nonmetallic atoms including the nitrogen atom are not adjacent to each other.

10 Claims, No Drawings

SILVER HALIDE COLOR PHOTOGRAPHIC MATERIAL CONTAINING A MAGENTA COLOR IMAGE-FORMING COUPLER

FIELD OF THE INVENTION

The present invention relates to a silver halide color photographic material, and more particularly, to a silver halide color photographic material that forms a dye image which is stable against heat or light and in which no stain is likely to occur.

BACKGROUND OF THE INVENTION

As is well known, in color development following the image-wise exposure of a silver halide color photographic material, the oxidized product of an aromatic primary amine color developing agent enters into coupling reaction with a color former to form a color image composed of, for example, indophenol, indoaniline, indamine, azomethine, phenoxyazine, phenazine or other dyes similar thereto. In this photographic process, color reproduction is usually achieved by the subtractive process using a silver halide color photographic material wherein blue-, green- and red-sensitive silver halide emulsion layers contain color formers, or couplers that will develop colors which are the respective complements of blue, green and red, namely, yellow, magenta and cyan colors.

An illustrative coupler used to form a yellow color image is acylacetanilide compound. Exemplary magenta image forming couplers include pyrazolone, pyrazolobenzimidazole, pyrazolotriazole and indazolone compounds. Among the couplers commonly used for cyan image formation are included phenolic and naphtholic compounds.

The dye image formed by the coupling reaction with such color formers and the oxidation product of aromatic primary amine color developing agent are required to undergo no discoloration or fading even if they are exposed to light or stored under hot and humid atmosphere for a prolonged period. It is also required that the background of a silver halide color photographic material (to be hereunder referred to simply as a color photographic material) or the areas where no color has formed should not undergo any yellow staining (hereunder Y staining) as a result of exposure to light or moist heat.

Magenta couplers are much more sensitive than yellow and cyan couplers to Y staining in the background caused by heat or moist heat as well as to the fading of the image areas resulting from prolonged exposure to light, and this has often caused serious problems in conventional color photography.

Couplers extensively used for magenta dye formation are 1,2-pyrazolo-5-ones. Dyes produced from such compounds generally have primary absorption at about 550 nm but they also have secondary absorption at about 430 nm. In order to minimize such secondary absorption, various efforts have been made. For example magenta couplers having an anilino group at 3-position of 1,2-pyrazolo-5-ones have relatively small degree of secondary absorption and are particularly useful for obtaining color image in print format. Details of this technique are found in U.S. Pat. No. 2,343,703 and British Pat. No. 1,059,994. However, such substituted magenta couplers are very poor in image keeping quality, especially in the fastness of color image to light. In

addition, the background is highly sensitive to Y staining.

Other magenta couplers that have been proposed as means capable of reducing the secondary absorption at about 430 nm include pyrazolobenzimidazoles (British Pat. No. 1,047,612), indazolones (U.S. Pat. No. 3,770,447) and pyrazolotriazoles (U.S. Pat. No. 3,725,067 and British Pat. Nos. 1,252,418 and 1,334,515). Dyes formed from the 1H-pyrazolo-[3,2-C]-s-triazole type couplers described in U.S. Pat. No. 3,725,067 and British Pat. Nos. 1,252,418 and 1,334,515 are preferred in terms of color reproduction over dyes formed from the 1,2-pyrazolo-5-ones having an anilino group at 3-position because the former has a far smaller secondary absorption at about 430 nm. Furthermore, the background of photographic materials using the 1H-pyrazolo-[3,2-C]-s-triazole type couplers as magenta couplers has extremely low sensitivity to Y staining resulting from exposure to light, heat or moisture.

However, the azomethine dye formed from the 1H-pyrazolo-[3,2-C]-s-triazole type couplers has a very small degree of fastness to light. In addition, such azomethine dye is highly likely to discolor upon exposure to light and has yet to be used commercially in color photographic materials, especially in color prints which are subject to considerable degradation resulting from the discoloration of azomethine dyes.

Unexamined Published Japanese Patent Application

No. 125732/1984 proposes a technique for improving the light fastness of the magenta dye image from the 1H-pyrazolo-[3,2-C]-s-triazole type coupler by using it in combination with a phenolic compound or a phenyl ether compound. However, even this technique is not completely satisfactory in preventing the magenta dye image from fading upon exposure to light, and is practically incapable of preventing the light discoloration of such dye image.

SUMMARY OF THE INVENTION

One object, therefore, of the present invention is to provide a color photographic material that is capable of faithful color reproduction and which exhibits a highly improved light fastness in magenta dye image.

Another object of the invention is to provide a color photographic material producing a magenta dye image that experiences a minimal degree of discoloration upon exposure to light.

A further object of the invention is to provide a color photographic material that is protected against the occurrence of Y stain in the background resulting from exposure to light or moist heat.

These objects of the invention can be achieved by a silver halide color photographic material containing a magenta color image-forming coupler represented by the following formula (I) and a compound represented by the following formula (II):



wherein

Z represents the group of nonmetallic atoms necessary for forming a nitrogen-containing heterocy-

clic ring, provided that the ring to be formed by said Z may have a substituent; X represents a hydrogen atom or a substituent capable of leaving upon reaction with the oxidized product of a color developing agent; and R represents a hydrogen atom or a substituent.



wherein R<sub>1</sub> is an aliphatic group, a cycloalkyl group or an aryl group; and

Y represents the group of nonmetallic atoms necessary for forming a 5- to 7-membered heterocyclic ring taken together with the nitrogen atom, provided that at least two hetero atoms among the heterocyclic ring-forming nonmetallic atoms including the nitrogen atom are not adjacent to each other.

In the magenta coupler of formula (I), the substituent represented by R includes, for example, a halogen atom, an alkyl group, a cycloalkyl group, an alkenyl group, a cycloalkenyl group, an alkinyl group, an aryl group, a heterocyclic group, an acyl group, a sulfonyl group, a sulfinyl group, a phosphonyl group, a carbamoyl group, a sulfamoyl group, a cyano group, a spirocompound residue, a bridged hydrocarbon compound residue, an alkoxy group, an aryloxy group, a heterocyclic oxy group, a siloxy group, an acyloxy group, a carbamoyloxy group, an amino group, an acylamino group, a sulfonamide group, an imido group, a ureido group, a sulfamoylamino group, an alkoxy carbonylamino group, an aryloxycarbonylamino group, an alkoxy carbonyl group, an aryloxycarbonyl group, an alkylthio group, an arylthio group and a heterocyclicthio group.

The halogen atom includes, for example, chlorine and bromine atoms, the chlorine atom being particularly preferable.

The alkyl group represented by R is preferably one having 1 to 32 carbon atoms, the alkenyl group and the alkinyl group are preferably those having 2 to 32 carbon atoms, and the cycloalkyl group and the cycloalkenyl group are preferably those having 3 to 12, particularly 5 to 7, carbon atoms, the alkyl, alkenyl and alkinyl groups each including those having a straight or branched chain.

These alkyl, alkenyl, alkinyl, cycloalkyl and cycloalkenyl groups each may have one or more substituents. Such substituents include, in addition to an aryl group, a cyano group, a halogen atom, a heterocyclic group, a cycloalkyl group, a cycloalkenyl group, a spiro-compound residue and a bridged hydrocarbon compound residue, for example, those substituted through the carbonyl group, such as acyl, carboxy, carbamoyl, alkoxy carbonyl and aryloxycarbonyl groups, and those substituted through the hetero atom, for example, those substituted through the oxygen atom, such as hydroxy, alkoxy, aryloxy, heterocyclic oxy, siloxy, acyloxy and carbamoyloxy groups, those substituted through the nitrogen atom, such as nitro, amino (including dialkylamino and the like), sulfamoylamino, aryloxycarbonylamino, aryloxycarbonylamino, acylamino, sulfoneamido, imido and ureido groups, those substituted through the sulfur atom, such as alkylthio, arylthio, heterocyclicthio, sulfonyl, sulfinyl and sulfamoyl groups, and those substi-

tuted through the phosphorus atom, such as a phosphonyl group and the like.

Examples of the alkyl group represented by R include, for example, methyl, ethyl, isopropyl, t-butyl, pentadecyl, heptadecyl, 1-hexyl nonyl, 1,1'-dipentyl nonyl, 2-chloro-t-butyl, trifluoromethyl, 1-ethoxytridecyl, 1-methoxyisopropyl, methanesulfonyl ethyl, 2,4-di-t-amylphenoxy methyl, anilino, 1-phenylisopropyl, 3-m-butanesulfonaminophenoxypropyl, 3-4'-{ $\alpha$ -[4'-(p-hydroxybenzenesulfonyl)phenoxy]dodecanoylamino}phenylpropyl, 3-{4'-[ $\alpha$ -(2',4'-di-t-amylphenoxy)butane amido phenyl]-propyl, 4-[ $\alpha$ -(O-chlorophenoxy)tetradecanamido phenoxy]-propyl, allyl, cyclopentyl and cyclohexyl groups.

The aryl group represented by R is preferably a phenyl group, and may have a substituent such as an alkyl, alkoxy or acylamino group.

Examples of the aryl group include phenyl, 4-t-butylphenyl, 2,4-di-t-amylphenyl, 4-tetradecaneamido phenyl, hexadecyl-oxyphenyl and 4'-[ $\alpha$ -(4'-t-butylphenoxy)tetradecaneamido]phenyl groups.

The heterocyclic group represented by R is preferably a 5- to 7-membered heterocyclic ring, and may be substituted or may be condensed. Examples of the heterocyclic group include 2-furyl, 2-thienyl, 2-pyrimidinyl and 2-benzothiazonyl groups.

The acyl group represented by R includes, for example, an alkylcarbonyl group such as acetyl, phenylacetyl, dodecanoyl and  $\alpha$ -2,4-di-t-amylphenoxybutanoyl groups, and an arylcarbonyl group such as benzoyl, 3-pentadecycloxybenzoyl and p-chlorobenzoyl groups.

The sulfonyl group represented by R includes, for example, an alkylsulfonyl group such as methylsulfonyl and dodecylsulfonyl groups, and an arylsulfonyl group such as benzenesulfonyl and p-toluenesulfonyl groups.

The sulfinyl group represented by R includes, for example, an alkylsulfinyl group such as ethylsulfinyl, octylsulfinyl and 3-fenoxybutylsulfinyl groups and an arylsulfinyl group such as phenylsulfinyl and m-pentadecylphenylsulfinyl groups.

The phosphonyl group represented by R includes, for example, an alkylphosphonyl group such as butyloxycetyl phosphonyl group, an alkoxyphosphonyl group such as octyloxyphosphonyl group, an aryloxyphosphonyl group such as phenoxyphosphonyl group and an arylphosphonyl group such as phenylphosphonyl group.

The carbamoyl group represented by R includes, for example, those substituted with an alkyl or aryl (preferably phenyl) group, such as, N-methylcarbamoyl, N,N-dibutylcarbamoyl, N-(2-pentadecyloctyl)carbamoyl, N-ethyl-N-dodecylcarbamoyl and N-[3-(2,4-di-t-amylphenoxy)-propyl]carbamoyl group.

The sulfamoyl group represented by R includes, for example, those substituted with an alkyl or aryl (preferably phenyl) group, such as N-propylsulfamoyl, N,N-diethylsulfamoyl, N-(2-pentadecyloxyethyl)sulfamoyl, N-ethyl-N-dodecylsulfamoyl and N-phenylsulfamoyl groups.

The spiro-compound residue represented by R includes, for example spiro[3,3]heptan-1-yl and the like.

The bridged hydrocarbon compound residue represented by R includes, for example, bicyclo[2,2,1]heptane-1-yl, tricyclo[3,3,1,1<sup>3,7</sup>]decane-1-yl and 7,7-dimethyl-1-bicyclo[2,2,1]heptane-1-yl.

The alkoxy group represented by R includes, for example, those substituted further with such a substituent(s) as is shown above with the alkyl group, such as me-

thoxy, propoxy, 2-ethoxyethoxy, pentadecyloxy, 2-dodecyloxyethoxy and phenethyloxyethoxy.

The aryloxy group represented by R is preferably a phenoxy group, and includes, for example, those of which aryl nucleus is further substituted with such a substituent(s) or an atom(s) as is shown above with the aryl group, such as phenoxy, p-t-butylphenoxy and m-pentadecylphenoxy groups.

The heterocyclicoxy group represented by R is preferably one having a 5- to 7-membered heterocyclic ring, and includes those of which heterocyclic ring has a substituent, such as 3,4,5,6-tetrahydropyran-2-oxy and 1-phenyltetrazole-5-oxy groups.

The siloxy group represented by R includes those substituted with an alkyl group, for example, trimethylsiloxy, triethylsiloxy and dimethylbutylsiloxy groups.

The acyloxy group represented by R includes, for example, alkylcarbonyloxy and arylcarbonyloxy groups, and further includes those having a substituent(s) such as acetoxy,  $\alpha$ -chloroacetoxy and benzoxyloxy groups.

The carbamoyloxy group represented by R includes those substituted with an alkyl or aryl group, such as N-ethylcarbamoyloxy, N,N-diethylcarbamoyloxy and N-phenylcarbamoyloxy groups.

The amino group represented by R includes those substituted with an alkyl or aryl (preferably phenyl) group, such as ethylamino, anilino, m-chloroanilino, 3-pentadecyloxycarbonylanilino and 2-chloro-5-hexadecaneamidoanilino groups.

The acylamino group represented by R includes alkylcarbonylamino and arylcarbonylamino (preferably phenylcarbonylamino) groups, and further includes those having a substituent(s) such as acetamido,  $\alpha$ -ethylpropaneamido, N-phenylacetamido, dodecaneamido, 2,4-di-t-amyloxyacetamido and  $\alpha$ -3-t-butyl-4-hydroxyphenoxybutaneamido groups.

The sulfonamido group represented by R includes alkylsulfonylamino and arylsulfonylamino groups, and further includes those having a substituent(s), such as 40 methylsulfonylamino, pentadecylsulfonylamino, benzensulfonamido, p-toluenesulfonamido and 2-methoxy-5-t-amylobenzenesulfonamido groups.

The imido group represented by R includes those which are open-chained or close-chained, and further 45 includes those having a substituent(s), such as, succinimido, 3-heptadecylsuccinimido, phthalimido and glutarimido groups.

The ureido group represented by R includes those substituted with an alkyl or aryl (preferably phenyl) group, such as N-ethylureido, N-methyl-N-decylureido, N-phenylureido and N-p-tolylureido groups.

The sulfamoylamino group represented by R includes those substituted with an alkyl or aryl (preferably phenyl) group, such as N,N-dibutylsulfamoylamino, 55 N-methylsulfamoylamino and N-phenylsulfamoylamino groups.

The alkoxy carbonylamino group represented by R includes those having a substituent(s), such as methoxycarbonylamino, methoxyethoxycarbonylamino and octadecyloxycarbonylamino groups.

The aryloxycarbonylamino group represented by R includes those having a substituent(s), such as phenoxy carbonylamino and 4-methylphenoxy carbonylamino groups.

The alkoxy carbonyl group represented by R includes those having a substituent(s), such as methoxycarbonyl,

butyloxycarbonyl, dodecyloxycarbonyl, octadecyloxycarbonyl, ethoxymethoxycarbonyloxy and benzyloxycarbonyl groups.

The aryloxycarbonyl group represented by R includes those having a substituent(s), such as phenoxy carbonyl, p-chlorophenoxy carbonyl and m-pentadecyloxyphenoxy carbonyl groups.

The alkylthio group represented by R includes those having a substituent(s), such as ethylthio, dodecylthio, octadodecylthio, phenethylthio and 3-phenoxypropylthio groups.

The arylthio group represented by R is preferably a phenylthio group, and includes those having a substituent(s), such as phenylthio, p-methoxyphenylthio, 2-t-octylphenylthio, 3-octadecylphenylthio, 2-carboxyphenylthio and p-acetaminophenylthio groups.

The heterocyclicthio group, represented by R is preferably a 5- to 7-membered heterocyclicthio group, and includes those having a condensed ring or having a substituent(s). Examples of such heterocyclicthio group include 2-pyridylthio, 2-benzothiazolylthio and 2,4-diphenoxyl-1,3,5-triazol-6-thio groups.

The substituent represented by X that is capable of leaving upon reaction with the oxidized product of a color developing agent includes, for example, those substituted through the carbon, oxygen, sulfur or nitrogen atom other than the halogen atom (chlorine, bromine or fluorine atom).

The groups which are substituted through the carbon atom include, in addition to the carboxyl group, a group represented by the following formula:



(wherein R<sub>1</sub>' is the same in meaning as said R; Z' is the same in meaning as said Z; and R<sub>2</sub>' and R<sub>3</sub>' each represents a hydrogen atom, an aryl, alkyl or heterocyclic group, a hydroxymethyl group and a triphenylmethyl group).

The groups which are substituted through the oxygen atom include, for example, alkoxy, aryloxy, heterocyclicoxy, acyloxy, sulfonyloxy, alkoxy carbonyloxy, aryloxycarbonyloxy, alkyloxycarbonyloxy and alkoxyoxycarbonyloxy groups.

The alkoxy group includes those having a substituent(s), such as ethoxy, 2-phenoxyethoxy, 2-cyanoethoxy, phenethyloxy, and p-chlorobenzyloxy groups.

The aryloxy group is preferably a phenoxy group, and includes those having a substituent(s). Examples of such aryloxy group include phenoxy, 3-methylphenoxy, 3-dodecylphenoxy, 4-methanesulfoneamidophenoxy, 4-[ $\alpha$ -(3'-pentadecylphenoxy)butaneamido]phenoxy, hexadecylcarbamoylmethoxy, 4-cyanophenoxy, 4-methanesulfonylphenoxy, 1-naphthylmethoxy and p-methoxyphenoxy groups.

The heterocyclicoxy group is preferably a 5- to 7-membered heterocyclicoxy group, and may be a condensed ring or include those having a substituent(s). Examples of such heterocyclicoxy group include 1-phenyltetrazolylmethoxy and 2-benzothiazolylmethoxy groups.

The acyloxy group includes, for example, an alkylcarbonyloxy group such as acetoxy and butanoyloxy

groups, an alkenylcarbonyloxy group such as a cinamoyloxy group, and an arylcarbonyloxy group such as a benzyloxy group.

The sulfonyloxy group includes, for example, butane-sulfonyloxy and methanesulfonyloxy groups.

The alkoxy carbonyloxy group includes, for example, ethoxycarbonyloxy and benzyloxycarbonyloxy groups.

The aryloxycarbonyloxy group includes a phenoxy carbonyloxy group and the like.

The alkyloxycarbonyloxy group includes, for example, a methyloxycarbonyloxy group.

The alkoxyoxalyl group includes an ethoxyoxalyl group and the like.

The group which is substituted through the sulfur atom includes, for example, alkylthio, arylthio, heterocyclicthio and alkyloxythiocarbonylthio groups.

The alkylthio group includes butylthio, 2-cyanoethylthio, phenethylthio and benzylthio groups.

The arylthio group includes phenylthio, 4-methanesulfoneamidophenylthio, 4-dodecylphenetylthio, 4-nonafluoropentaneamidophenetylthio, 4-carboxyphenylthio and 2-ethoxy-5-t-butylphenylthio groups.

The heterocyclicthio group includes, for example, 1-phenyl-1,2,3,4-tetrazolyl-5-thio and 2-benzothiazolylthio groups.

The alkyloxythiocarbonylthio group includes a dodecyloxythiocarbonylthio group and the like.

The group which is substituted through the nitrogen atom includes, for example, one represented by the formula



wherein R<sub>4'</sub> and R<sub>5'</sub> each represents a hydrogen atom, an alkyl, aryl, heterocyclic, sulfamoyl, carbamoyl, acyl, sulfonyl, aryloxycarbonyl or alkoxy carbonyl group, and R<sub>4'</sub> and R<sub>5'</sub> may cooperate to form a heterocyclic ring, provided that R<sub>4'</sub> and R<sub>5'</sub> are not hydrogen atoms at the same time.

The alkyl group may be straight-chained or branched and is preferably one having 1 to 22 carbon atoms. Also, the alkyl group may include those having a substituent(s). Examples of such substituent include, for example, aryl, alkoxy, aryloxy, alkylthio, arylthio, alkylamino, arylamino, acylamino, sulfoneamido, imino, acyl, alkylsulfonyl, arylsulfonyl, carbamoyl, sulfamoyl, alkoxy carbonyl, aryloxycarbonyl, alkyloxycarbonyl amino, aryloxycarbonyl amino, hydroxy, carboxyl and ciano groups and halogen atom. Examples of such alkyl group includes, for example, ethyl, octyl, 2-ethylhexyl and 2-chloroethyl group.

The aryl group represented by R<sub>4'</sub> or R<sub>5'</sub> is preferably one having 6 to 32 carbon atoms, particularly a phenyl or naphtyl group, and may include those having a substituent(s). Such substituent includes a substituent for the alkyl group represented by R<sub>4'</sub> or R<sub>5'</sub> and an alkyl group. Examples of the aryl group include, for example, phenyl, 1-naphtyl and 4-methylsulfonylphenyl groups.

The heterocyclic group represented by R<sub>4'</sub> or R<sub>5'</sub> is preferably a 5- or 6-membered ring, and may be a condensed ring or include those having a substituent(s). Examples of such heterocyclic group include 2-furyl,

2-quinolyl, 2-pyrimidyl, 2-benzothiazolyl and 2-pyridyl groups.

The sulfamoyl group represented by R<sub>4'</sub> or R<sub>5'</sub> includes N-alkylsulfamoyl, N,N-dialkylsulfamoyl, N-arylsulfamoyl and N,N-diarylsulfamoyl groups, and these alkyl and aryl groups may have such a substituent(s) as is mentioned with respect to the alkyl and aryl groups. Examples of such sulfamoyl group includes, for example, N,N-diethylsulfamoyl, N-methylsulfamoyl, N-dodecylsulfamoyl and N-p-tolylsulfamoyl groups.

The carbamoyl group represented by R<sub>4'</sub> or R<sub>5'</sub> includes N-alkylcarbamoyl, N,N-dialkylcarbamoyl, N-arylcaramoyl and N,N-diarylcaramoyl groups, and

15 these alkyl and aryl groups may have such a substituent(s) as is mentioned with respect to the alkyl and aryl groups. Examples of such carbamoyl group include, for example, N,N-diethylcarbamoyl, N-methylcarbamoyl, N-dodecylcarbamoyl, N-p-cianophenylcarbamoyl and N-p-tolylcarbamoyl groups.

The acyl group represented by R<sub>4'</sub> or R<sub>5'</sub> includes, for example, alkylcarbonyl, arylcarbonyl and heterocyclic carbonyl groups, and the alkyl, aryl and heterocyclic groups may have a substituent(s). Examples of such acyl group include, for example, hexafluorobutanoyl, 2,3,4,5,6-pentafluorobenzoyl, acetyl, benzoyl, naphtoyl and 2-furylcarbonyl groups.

The sulfonyl group represented by R<sub>4'</sub> or R<sub>5'</sub> includes alkylsulfonyl, arylsulfonyl and heterocyclicsulfonyl groups, and may have a substituent(s). Examples of such sulfonyl group include, for example, ethanesulfonyl, benzenesulfonyl, octanesulfonyl, naphthalenesulfonyl and p-chlorobenzenesulfonyl groups.

The aryloxycarbonyl group represented by R<sub>4'</sub> or R<sub>5'</sub> 35 may have such a substituent(s) as is mentioned with respect to the aryl group, and includes a phenoxy carbonyl group and the like.

The alkoxy carbonyl group represented by R<sub>4'</sub> or R<sub>5'</sub> 40 may have such a substituent(s) as is mentioned with respect to alkyl group, and includes methoxycarbonyl, dodecyloxy carbonyl and benzyl oxycarbonyl groups.

The heterocyclic ring which is formed through cooperation of R<sub>4'</sub> and R<sub>5'</sub> is preferably a 5- or 6-membered ring, may be saturated or unsaturated, may or may not be an aromatic ring, or may be a condensed ring. Examples of such heterocyclic ring include, for example, N-phthalimido, N-succinimide, 4-N-urazolyl, 1-N-hydantoinyl, 3-N-2,4-dioxoazolidinyl, 2-N-1,1-dioxo-3-(2H)-oxo-1,2-benzthiazolyl, 1-pyrrolyl, 1-pyrrolidinyl, 1-pyrazolyl, 1-pyrazolidinyl, 1-piperidinyl, 1-pyrrolinyl, 1-imidazolyl, 1-imidazolinyl, 1-indolyl, 1-isindolinyl, 2-iso-indolyl, 2-isoindolinyl, 1-benzotriazolyl, 1-benzoimidazolyl, 1-(1,2,4-triazolyl), 1-(1,2,3-triazolyl), 1-(1,2,3,4-tetrazolyl), N-morpholinyl, 1,2,3,4-tetrahydroquinolyl, 2-oxo-1-pyrrolidinyl, 2-1H-pyridone, phthalazione and 2-oxo-1-piperidinyl groups. These heterocyclic groups may be substituted by alkyl, aryl, alkyloxy, aryloxy, acyl, sulfonyl, alkylamino, arylamino, acylamino, sulfoneamino, carbamoyl, sulfamoyl, alkylthio, arylthio, ureido, alkoxy carbonyl, aryloxycarbonyl, imido, nitro, cyano, carboxyl groups as well as by a halogen atom and the like.

The nitrogen-containing heterocyclic ring which is formed by Z or Z' includes pyrazol, imidazol, triazol and tetrazol rings, and may have such a substituent(s) as is mentioned with respect to R.

When the substituent(s) (for example either of R and R<sub>1</sub> to R<sub>8</sub>) on the heterocyclic ring in formula (I) and in

formulas (III) to (IX) to be mentioned later has the following formula:



(wherein R'', X and Z'' are the same in meaning as R, X and Z in formula (I), respectively), the coupler formed is the so-called bis-type coupler, which is included in the present invention. The ring which is formed by Z, Z', Z'' as well as by Z<sub>1</sub> to be stated later may be condensed with another ring (for example 5- to 7-membered cycloalkene). For example, in formula (VI), R<sub>5</sub> and R<sub>6</sub>, and in formula (VII), R<sub>7</sub> and R<sub>8</sub>, may cooperate to form a ring (for example, 5- to 7-membered cycloalkene, or benzene), respectively.

The coupler represented by formula (I) preferably includes, for example, those represented by the following formulas (III) to (VIII):



wherein R<sub>1</sub> to R<sub>8</sub> and X are the same in meaning as R and X mentioned above.

The coupler of formula (I) is preferably one represented by the following formula (IX):



wherein R<sub>1</sub>, X and Z<sub>1</sub> are the same in meaning as R, X and Z in formula (I).

Of the magenta couplers represented by formulas (III) to (VIII), those represented by formula (III) are particularly preferable.

With respect to the substituent(s) on the heterocyclic ring in formulas (I) and (II) to (IX), R in formula (I) and R<sub>1</sub> in formulas (III) to (IX) are preferable when they satisfy the following requirement 1, the same R and R<sub>1</sub> are more preferable when they satisfy the following requirements 1 and 2, and the same R and R<sub>1</sub> are most preferable when they satisfy all of the following requirements 1, 2 and 3:

Requirement 1: The root atom bonded directly to the heterocyclic ring is a carbon atom.

Requirement 2: Said carbon atom has only one hydrogen atom or has no hydrogen atom at all, bonded thereto.

Requirement 3: The bonds between said carbon atom and adjacent atoms are all single bonds.

The most preferable substituents R and R<sub>1</sub> on the heterocyclic ring are those represented by the following formula (X):



(III) 25

(IV)

(V)

(VI)

(VII)

(VIII)

30

35

40

45

50

55

60

65

65

wherein R<sub>9</sub>, R<sub>10</sub> and R<sub>11</sub> each represents a hydrogen atom, a halogen atom, an alkyl group, a cycloalkyl group, an alkenyl group, a cycloalkenyl group, an alkynyl group, an aryl group, a heterocyclic group, an acyl group, a sulfonyl group, a sulfinyl group, a phosphoryl group, carbamoyl group, a sulfamoyl group, a cyano group, a spiro-compound residue, a bridged hydrocarbon compound residue, an alkoxy group, an aryloxy group, a heterocyclicoxy group, a siloxy group, an acyloxy group, a carbamoyloxy group, an amino group, an acylamino group, a sulfonamide group, an imido group, a ureido group, a sulfamoyl amino group, an alkoxy carbonyl amino group, an aryloxy carbonyl amino group, an alkoxy carbonyl group, an aryloxy carbonyl group, an alkylthio group, an arylthio group or a heterocyclithio group, provided that at least two of R<sub>9</sub>, R<sub>10</sub> and R<sub>11</sub> are not hydrogen atoms.

Two of R<sub>9</sub>, R<sub>10</sub> and R<sub>11</sub>, for example, R<sub>9</sub> and R<sub>10</sub> may cooperate to form a saturated or unsaturated ring (e.g. cycloalkane, cycloalkene or heterocyclic ring), and further R<sub>11</sub> may cooperate with said ring to form a bridged hydrocarbon compound residue.

The group represented by R<sub>9</sub> to R<sub>11</sub> may have a substituent(s). Examples of said group and said substituent(s) are the same as the examples of the group represented by R in formula (I) and the substituent(s) mentioned with respect thereto.

Examples of the ring formed by the cooperation of, for example, R<sub>9</sub> and R<sub>10</sub>, as well as of the bridged hydrocarbon compound residue which is formed by R<sub>9</sub> to R<sub>11</sub> and the substituent(s) which said residue may have, are the same as the examples of the cycloalkyl, cycloalkenyl, and heterocyclic groups represented by R in formula (I), and the substituent(s) mentioned with respect thereto.

The preferable substituents in formula (X) are as follows:

(i) Two of R<sub>9</sub> to R<sub>11</sub> are alkyl groups.

(ii) One of R<sub>9</sub> to R<sub>11</sub>, for example, R<sub>11</sub> is a hydrogen atom, and the other two, R<sub>9</sub> and R<sub>10</sub>, cooperate with the root carbon atom to form a cycloalkyl group.

Further, the preferable substituent(s) in (i) above is such that two of R<sub>9</sub> to R<sub>11</sub> are alkyl groups, and the other one is a hydrogen atom or an alkyl group.

The alkyl and cycloalkyl groups each may have a substituent(s). Examples of such alkyl and cycloalkyl groups as well as of their substituents are the same as the

examples of the alkyl and cycloalkyl groups represented by R in formula (I) and the substituents mentioned with respect thereto.

Typical, but by no means limiting, examples of the magenta color image-forming coupler that can be used in the present invention are listed below.

ILLUSTRATIVE MAGENTA COLOR  
IMAGE-FORMING COUPLERS

PC-1



PC-2



PC-3



PC-4



PC-5



PC-6



PC-7



-continued



PC-8



PC-9



PC-10



PC-11



PC-12



PC-13



PG-14



PC-15

-continued



-continued

PC-26



PC-27



PC-28



PC-29



PC-30



PC-31



PC-32



PC-33



-continued

PC-34



PC-35



PC-36



PC-37



PC-38



PC-39



PC-40



PC-41



-continued



PC-42



PC-44



PG-45



PC-46



PC-47



PC-48



PC-49

-continued

PC-50



PC-51



PC-52



PC-53



PC-54



PC-55



PC-56



PC-57



-continued



PC-58



PC-59



PC-60



PC-61



PC-62



PC-63



PC-64

4,639,415

27

28

-continued

PC-65



PC-66



PC-67



PC-68



PC-68



PC-69



PC-70



PC-71



PC-72



PC-73



-continued



PC-75



PC-76



PC-77



PC-79



PC-80



PC-81



PC-82



PC-83



-continued

PC-84



PC-85



PC-86



PC-87



PC-88



PC-89



PC-90



PC-91



PC-92



-continued

PC-93



PC-94



PC-95



PC-96



PC-97



PC-98



PC-99



PC-100



-continued

PC-101



PC-102



PC-103



PC-104



PC-105



PC-106



PC-107



PC-108



PC-109



PC-110

-continued

PC-111



PC-112



PC-113



PC-114



PC-115



PC-116



PC-117



PC-118



**-continued**

PC-119



PC-120



PC-121



PC-122



PC-123



PC-124



PC-125



-continued

PC-126



PC-127



PC-128



PC-129



PC-130



PC-131



PC-132



PC-133



PC-134



PC-135



PC-136

-continued

PC-137



PC-138



PC-139



PC-140



PC-141



PC-142



-continued



PC-143



PC-144



PC-145



PC-146



PC-147



PC-148



PC-149



PC-150



PC-151

-continued



PC-153



PC-155



PC-156



PC-157



PC-158



PC-159



PC-160



PC-161



PC-162

-continued





-continued  
PC-172



These couplers were synthesized by reference to Journal of the Chemical Society, Perkin I (1977), pages 2047 to 2052, U.S. Pat. No. 3,725,067 and Unexamined Published Japanese Patent Application Nos. 99437/1984, 42045/1983, 162548/1984, 59171956/1984, 33552/1985 and 43659/1985.

A magenta dye image stabilizer having the formula (I) which is used in combination with the magenta coupler of the present invention has the effect of not only preventing a magenta dye image from fading upon exposure to light but also preventing light discoloration of said image.

In formula (II), R' represents an aliphatic group, a cycloalkyl group or an aryl group, and these may have substituents. Examples of the aliphatic group represented by R' include saturated and unsaturated alkyl groups. Illustrative saturated aliphatic groups include methyl, ethyl, butyl, octyl, dodecyl, tetradecyl and hexadecyl. Exemplary unsaturated aliphatic groups include ethenyl and propenyl.

Examples of the cycloalkyl group represented by R' include optionally substituted 5- to 7-membered cycloalkyl groups such as cyclopentyl and cyclohexyl.

Examples of the aryl group represented by R' are a phenyl and naphthyl that may have a substituent.

Examples of the substituent for the aliphatic group, cycloalkyl group and aryl group represented by R' include alkyl, aryl, alkoxy, carbonyl, carbamoyl, acylamino, sulfamoyl, sulfonamido, carbonyloxy, alkylsulfonyl, arylsulfonyl, hydroxyl, hetero ring, alkylthio and arylthio. These substituents may be optionally substituted.

In formula (II), Y represents the group of nonmetallic atoms necessary for forming a 5- to 7-membered hetero ring taken together with the nitrogen atom. At least two of the hetero ring forming nonmetallic atoms including the nitrogen atom must be hetero atoms and these two hetero atoms should not be adjacent to each other. Compounds of formula (II) having two adjacent hetero atoms in the hetero ring are not desirable since they are not effective as the magenta dye image stabilizer.

The 5- to 7-membered hetero ring in the compounds of formula (II) may have a substituent such as an alkyl or aryl group. The 5- to 7-membered hetero ring may be saturated or unsaturated but a saturated hetero ring is preferred.

Typical, but by no means limiting, examples of the compounds of formula (II) are listed below.

#### EXEMPLARY COMPOUNDS OF FORMULA (II)

##### (A) Piperazine compounds:



A-1



A-3



A-5



A-7



A-9



A-11



A-13



A-15



A-17



A-19



A-21



A-22



A-23





-continued

A-24



A-25

A-26



A-27



A-28



A-29



A-30



(B) Morpholine compounds:

-continued



B-1

B-2



B-2



B-3

B-4



B-5

B-6



B-7

B-8



B-8

B-9



B-10

(C) Thiamorpholine compounds:



C-1

65



C-2



-continued



**(D) Imidazolidine compounds:**



### (E) Homopiperazine compounds:



4,639,415

58

-continued



15. (H) Others:



-continued



Among the magenta dye image stabilizers of formula (11) used in the present invention, piperazine and homopiperazine compounds are particularly preferred. Among the piperazine and homopiperazine compounds, those represented by the following formulas (XI) and (XII) are preferred:



wherein  $R^2$  is a hydrogen atom, an alkyl group or an aryl group  $R^3$  is a hydrogen atom, an alkyl group, an acyl group on an aryl group,  $R^3$  being preferably a hydrogen atom, an alkyl group or an aryl group, provided that  $R^2$  and  $R^3$  are not both hydrogen atoms; and  $R^4$  to  $R^{13}$  are each a hydrogen atom, an alkyl group or an aryl group.

In formulas (XI) and (XII),  $R^2$  represents a hydrogen atom, an alkyl group or an aryl group; and  $R^3$  represents a hydrogen atom, an alkyl group, an acyl group or an aryl group. Examples of the alkyl group represented by  $R^2$  or  $R^3$  include methyl, ethyl, butyl, octyl, dodecyl, tetradecyl, hexadecyl and octadecyl. Examples of the acyl group represented by  $R^3$  include an alkyl carbonyl group such as acetyl, dodecanoyl and the like, and an aryl carbonyl group such as benzoyl and the like. An example of the aryl group represented by  $R^2$  or  $R^3$  is a phenyl group. The alkyl group and aryl group represented by  $R^2$  or  $R^3$  may have a substituent such as a halogen atom, an alkyl group, an aryl group, an alkoxy group, an aryloxy group or a heterocyclic group.

The sum of carbon atoms in  $R^2$  and  $R^3$  (including substituents) is preferably in the range of 6 to 40. In formula (XI) and (XII),  $R^4$  to  $R^{13}$  each represents a hydrogen atom, an alkyl group or an aryl group. Examples of the alkyl group represented by  $R^4$  to  $R^{13}$  include methyl and ethyl. An example of the aryl group represented by  $R^4$  to  $R^{13}$  is a phenyl group.

Specific examples of the compounds represented by formula (XI) have been listed above as illustrative piperazine compounds (A-1) to (A-30), while specific examples of the compounds represented by formula (XII) have been listed as illustrative homopiperazine compounds (E-1) to (E-12). Typical examples of the magenta dye image stabilizer having formula (11) used in the present invention may be synthesized by the following methods.

### SYNTHESIS 1

#### Synthesis of Compound (A-2):

Piperazine (9.0 g) and myristyl bromide (55 g) are dissolved in 100 ml of acetone. To the acetone solution, 15 g of anhydrous potassium carbonate is added and the mixture is refluxed for 10 hrs. After the reaction, the reaction mixture is poured into 500 ml of water and subjected to extraction with 500 ml of ethyl acetate. The ethyl acetate layer is dried over magnesium sulfate and the ethyl acetate is distilled off so as to obtain the end compound as a white crystal. The crystal is recrys-

tallized with 300 ml of acetone to obtain white flakes in an amount of 34 g (yield: 70%). m.p. 55°-58° C.

## SYNTHESIS 2

## Synthesis of Compound (B-4):

Eighteen grams of 4-morpholinoaniline is dissolved in 100 ml of ethyl acetate. To the stirred solution while held at 20° C., 12 ml of acetic anhydride is added in small portions. After completion of the addition of 10 acetic anhydride, the mixture is cooled with ice. The resulting crystal is recovered by filtration and recrystallized with ethyl acetate to obtain the end compound as a white powder in an amount of 16.5 g (yield: 75%). m.p. 207°-210° C. 15

The color photographic material of the present invention preferably contains the magenta coupler in amounts ranging from  $1.5 \times 10^{-3}$  to  $7.5 \times 10^{-1}$  moles per mole of silver, more preferably from  $1 \times 10^{-2}$  to 20  $5 \times 10^{-1}$  moles per mole of silver.

The magenta dye image stabilizer of formula (11) is preferably used in amounts ranging from 5 to 300 mole%, more preferably 10-200 mole%, of the magenta coupler of formula (I). 25

The magenta dye image stabilizer of formula (11) may be used in combination with another magenta dye image stabilizer that is represented by the following formula (XIII), namely a phenolic or phenylether compound: 30



wherein R<sup>14</sup> is a hydrogen atom, an alkyl group, an aryl group or a heterocyclic group; R<sup>15</sup>, R<sup>16</sup>, R<sup>18</sup> and R<sup>19</sup> are each a hydrogen atom, a hydroxyl group, an alkyl group, an aryl group, an alkoxy group or an acylamino group; R<sup>17</sup> is an alkyl group, a hydroxyl group, an aryl group or an alkoxy group; R<sup>14</sup> and R<sup>15</sup> may be fused to form a 5- or 6-membered ring when R<sup>17</sup> represents a hydroxy or alkoxy group; R<sup>14</sup> and R<sup>15</sup> may be fused to form a methylenedioxy ring; and R<sup>16</sup> and R<sup>17</sup> may be fused to form a 5-membered carbon ring when R<sup>14</sup> represents an alkyl, aryl or heterocyclic group. 45

Several of the compounds of formula (XIII) are described in U.S. Pat. Nos. 3,935,016, 3,982,944, and 4,254,216; Unexamined Published Japanese Patent Application Nos. 21004/1980 and 145530/1979; Published British Patent Application Nos. 2,077,455 and 2,062,888; U.S. Pat. Nos. 3,764,337, 3,432,300, 3,574,627 and 3,573,050; Unexamined Published Japanese Patent Application Nos. 152225/1977, 20327/1978, 17729/1978 and 6321/1980; British Pat. No. 1,347,556; Published British Patent Application No. 2,066,975; Japanese Patent Publication Nos. 12337/1979 and 31625/1973; and U.S. Pat. No. 3,700,455. 60

Specific examples of the compounds of formula (XIII) are listed below. 65





10 The phenolic or phenylether compound of formula (XIII) is preferably used in an amount not more than 200 mole% of the magenta dye image stabilizer of formula (II), with the amount not exceeding 140 mole% being more preferred.

15 The phenolic compound and phenylether compound of formula (XIII) are effective in preventing the fading of the magenta dye produced from the magenta coupler of the present invention, but they are little effective in preventing such magenta dye image from becoming discolored. Therefore, it is not preferred that the phenolic or phenylether compound is used in an excess amount with respect to the magenta dye image stabilizer of formula (II).

20 The magenta dye image formed from the magenta coupler of the present invention generally undergoes considerable fading upon exposure to light. Furthermore, discoloration resulting from exposure to light is so great that the color of the image changes from the pure magenta to yellowish magenta. The magenta dye image stabilizer of formula (II) is capable of exhibiting the effects unattainable by the phenolic or phenylether compound, i.e., prevention of fading and discoloration of the magenta dye image produced from the magenta coupler used in the present invention.

25 Accordingly, when the magenta dye image stabilizer of formula (II) is used in admixture with the conventional magenta dye image stabilizer, i.e., phenolic or phenylether compound, said conventional stabilizer must be used in such an amount that the discoloration upon exposure to light is not remarkable.

30 When such conventional stabilizer, i.e., phenolic or phenylether compound, of formula (XIII) is used in a suitable amount in combination with the magenta dye image stabilizer of formula (II), a synergistic effect is sometimes observed which is due probably to their compensating for the mutual defective points each other.

35 The magenta coupler and magenta dye image stabilizer in accordance with the present invention are preferably used in the same photographic layer, but if desired, they may be incorporated in two different layers such that the stabilizer in a layer adjacent the one containing the magenta coupler.

40 The silver halide photographic material of the present invention may be, for example, color negative and positive films and color photographic paper, but particularly when color photographic paper for viewing the printed color image directly is used, the effect of the present invention is produced strikingly.

45 The silver halide photographic material of the present invention including such color photographic paper may be either for monochrome or multicolor use. The silver halide photographic material for multicolor use has a structure such that silver halide emulsion layers usually containing magenta, yellow and cyan couplers, respectively, as photographic couplers, and nonsensitive layers are superimposed in appropriate number of layers and in appropriate sequence on the support in

order to effect subtractive color reproduction, but such number of layers and sequence may be changed appropriately according to use object.

The silver halide emulsion used in the silver halide photographic material of the present invention may be selected from among the silver halides commonly used in silver halide photography, such as silver bromide, silver chloride, silver iodobromide, silver chlorobromide and silver chloroiodobromide.

The silver halide grains used in the silver halide emulsions of the present invention may be those obtained by any of the acid method, neutral method, and ammoniacal method. These grains may be grown at one time or may be grown after preparing seed grains. The method of preparing seed grains and the method of growing them may be the same or different.

In preparing the silver halide emulsion, halide ions and silver ions may admixed at the same time, or either one may be admixed with the other one present in the emulsion. Also, while considering the critical speed of growth of silver halide crystals, halide ions and silver ions may be added one by one or at the same time into a mixing bath while controlling the pH and pAg in said bath to grow the crystals.

In preparing the silver halide of the present invention, it is possible, by using a silver halide solvent optionally, to control the grain size, shape, grain size distribution and speed of growth of the silver halide grains.

The silver halide grains to be used in the silver halide emulsions of the present invention may have metal ions incorporated inside the grains and/or in the grain surfaces in the course of forming and/or growing the grains by using cadmium salt, zinc salt, lead salt, thallium salt, or iridium salt or its complex salt, rhodium salt or its complex salt, or iron salt or its complex salt. Said grains may also be placed in an appropriate reduction atmosphere to have reduction-sensitized specks imparted inside the grains and/or into the grain surfaces.

The silver halide emulsions of the present invention may be removed of unnecessary soluble salts after completion of the growth of the silver halide grains or may be left as they are containing such salts. In removing said salts; the method described in "Research Disclosure No. 17643" may be used.

The silver halide grains to be used in the silver halide emulsions of the present invention may have a homogeneous structure throughout the crystal, or the structure of the core may be different from that of the shell. These silver halide grains may be of the surface type where latent images are predominantly formed on the grain surface or of the internal type where latent images are formed within the grain.

The silver halide grains may be regular crystals or irregular crystals such as inspherical or plane form. They may have any proportions of (100) and (111) planes, and may also be in composite form of these crystals or may be admixed with various crystal grains.

The silver halide emulsion of the present invention may be a mixture of two or more silver halide emulsions prepared separately.

The silver halide emulsion of the present invention is chemically sensitized by an ordinary method, such as the sulfur sensitization using a compound containing sulfur capable of reaction with silver ions or using active gelatin, the selenium sensitization using a selenium compound, the reduction sensitization using reducible material, or the noble metal sensitization using gold and

other noble metal compounds. Such methods may be used each independently or in combination.

The silver halide emulsion of the present invention may be spectrally sensitized by suitably selected sensitizing dye in order to provide sensitivity for the desired spectral wavelength regions. A variety of spectral sensitizing dyes may be used either individually or in combination. The silver halide emulsion may contain, together with the sensitizer, a dye which itself has no spectral sensitizing action or a supersensitizer which, being a compound which substantially does not absorb visible light, strengthens the sensitizing action of the sensitizer.

In order to prevent the occurrence of fog and/or keep the photographic properties stable, in the course of preparing the photographic material, in storage or in processing thereof, a compound known in the photographic industry as an anti-foggant or stabilizer may be added to the silver halide emulsion of the present invention in the course of chemical ripening and/or upon completion of chemical ripening and/or after completion of chemical ripening but before coating of the silver halide emulsion.

The binder (or protective colloid) advantageously used in the silver halide emulsion of the present invention is gelatin, but other hydrophilic colloids such as gelatin derivative, graft polymer of gelatin with other polymer, protein, sugar derivative, cellulose derivative, and synthesized hydrophilic polymer may be used.

The photographic emulsion layer and other hydrophilic colloidal layer(s) of the photographic material using the silver halide emulsion of the present invention are hardened by using hardeners either alone or in combination that bridge the binder (or protective colloid) molecules to enhance the film strength. The hardener is desirably added in such an amount as is capable of hardening the photographic material to the extent that there is no need to add the hardener in the processing solution, but such hardener may be added in the processing solution.

A plasticizer can be added with a view to enhancing the flexibility of the silver halide emulsion layer and/or other hydrophilic colloidal layer(s) of the photographic material using the silver halide emulsion of the present invention.

A water-insoluble or hardly soluble synthesized polymer latex can be incorporated for the purpose of improving the dimensional stability of the photographic emulsion layer and other hydrophilic colloidal layer(s) of the photographic material using the silver halide emulsion of the present invention.

In the emulsion layer of the silver halide color photographic material of the present invention, a dye-forming coupler is used which forms a dye upon coupling reaction with the oxidized product of an aromatic primary amine developing agent (e.g., p-phenylenediamine derivative or aminophenol derivative) in the color developing processing. The color-forming coupler is usually selected so that a dye is formed which absorbs the spectral wavelength sensitive to the emulsion layer containing said dye; that is, a yellow dye-forming coupler is used in the blue-sensitive emulsion layer, a magenta dye-forming coupler in the green-sensitive emulsion layer, and a cyan dye-forming coupler in the red-sensitive emulsion layer. However, the respective couplers may be used in different combinations from those mentioned above according to the object.

The yellow dye-forming coupler includes acylacetamido couplers (e.g. benzoylacetanilides and pivaloyl acetanilides), the magenta dye-forming coupler includes, in addition to the couplers of the present invention, 5-pyrazolone, pyrazolobenzimidazole, pyrazolotriazole and open chained acylacetonitrile couplers, and the cyan dye-forming coupler includes naphthol and phenol couplers.

These dye-forming couplers desirably have a group having 8 or more carbon atoms in the molecule that, being called a ballast group, renders the coupler non-diffusible. These couplers may be 4-equivalent couplers such that four silver ions need be reduced for the formation of one mole of dye, or may be 2-equivalent couplers such that only two silver ions suffice to be reduced for the formation of one mole of dye.

Hydrophobic compounds such as dye-forming coupler that need not be adsorbed onto the silver halide crystal surfaces can be dispersed into the emulsion by means of solid dispersion, latex dispersion or oil-in-water drop type emulsion dispersion. Such dispersion method can be appropriately selected according to the chemical structure and the like of the hydrophobic compounds. The oil-in-water drop type emulsion dispersion method may be any conventional method of dispersing hydrophobic additives such as coupler, which usually comprises dissolving such hydrophobic additives in a high-boiling organic solvent having a boiling point higher than about 150° C. by optionally using low-boiling and/or water-soluble organic solvents together, then emulsion-dispersing the dissolved hydrophobic additives by using a surfactant in a hydrophilic binder such as aqueous gelatin solution with such means of dispersion as a stirrer, homogenizer, colloid mill, flow-jet mixer or ultrasonic disperser, and thereafter adding the resulting dispersion into the hydrophilic colloidal layer. In that case, the step of removing the low-boiling organic solvent after or simultaneously with dispersion may be added.

The high-boiling organic solvent is one having a boiling point higher than 150° C. that does not react with the oxidized product of a developing agent, such as a phenol derivative, phthalate ester, phosphate ester, citrate ester, benzoate ester, alkylamido, fatty acid ester or trimeric acid ester.

Dispersion aids used in dissolving hydrophobic compounds in a low-boiling solvent alone or mixed with a high-boiling solvent and dispersing the dissolved hydrophobic compounds into water by using a mixer or ultrasonic disperser include anionic surfactants, nonionic surfactants and cationic surfactants.

Anti-color foggants may be used in order to prevent occurrence of color stain, deterioration of sharpness and coarse graininess due to moving of the oxidized product of a developing agent or the electron transporting agent between the emulsion layers (the same color-sensitive layers and/or different color-sensitive layers) of the color photographic material of the present invention.

The anti-color foggants may be incorporated in the emulsion layer itself or in the intermediate layer provided between adjacent emulsion layers.

Image stabilizers can be incorporated in the color photographic material using silver halide emulsion layers of the present invention in order to prevent deterioration of color images.

The hydrophilic colloidal layers such as protective layer and intermediate layer of the photographic mate-

rial of the present invention may have incorporated therein UV absorbers in order to prevent occurrence of fogging due to discharge resulting from the photographic material being charged by its friction or the like, or to prevent deterioration of images due to UV light.

The color photographic material using a silver halide emulsion of the present invention can be provided with auxiliary layers such as filter layer, anti-halation layer and/or anti-irradiation layer. These auxiliary layers and/or the emulsion layers may have incorporated therein dyes flowing out of the color photographic material or being bleached during the color developing processing.

Matting agents can be incorporated in the silver halide emulsion layers and/or other hydrophilic colloidal layers of the silver halide photographic material using a silver halide emulsion of the present invention, with a view to reducing the surface gloss to render writing in pencil possible and to preventing adhesion of photographic materials to each other.

The light-sensitive material using the silver halide emulsion of the present invention may contain a lubricant that is capable of reducing its sliding friction.

The light-sensitive material may also contain an antistat for the purpose of preventing static buildup. The antistat may be incorporated in an antistatic layer on the side of the support where no emulsion layer is formed. Alternatively, the antistat may be incorporated in an emulsion layer and/or a protective layer other than an emulsion layer which is on the side of the support where said emulsion layer is formed.

Photographic emulsion layer and/or other hydrophilic colloidal layers in the light-sensitive material using the silver halide emulsion of the present invention may contain a variety of surfactants for attaining such purposes as improved coating property, prevention of antistatic buildup, improved slipping property emulsification/dispersing, antiblocking and improved photographic characteristics in terms of accelerated development, hard tone and sensitization.

Photographic emulsion layers and other layers for making a light-sensitive material using the silver halide emulsion of the present invention may be coated onto flexible reflecting supports such as paper or synthetic paper laminated with baryta layer or  $\alpha$ -olefin polymer, films made of semi-synthetic or synthetic polymers such as cellulose acetate, cellulose nitrate, polystyrene, polyvinyl chloride, polyethylene terephthalate, polycarbonate and polyamide, and rigid materials such as glass, metals and ceramics.

After optional surface treatment of the support by suitable techniques such as corona discharge, UV irradiation and flame treatment, the silver halide light-sensitive material of the present invention may be coated onto the support either directly or with one or more subbing layers formed thereon. The subbing layers are provided for improving the adhesive strength, antistatic property, dimensional stability, frictional resistance, hardness, anti-halation property, frictional characteristics and/or other characteristics of the surface of the support.

A thickener may be used in order to facilitate the coating of the photographic material using the silver halide emulsion of the present invention. Particularly useful coating techniques are extrusion coating and curtain coating, both of which will enable simultaneous application of two or more layers.

The light-sensitive material of the present invention may be exposed to electromagnetic waves in the spectral region to which the emulsion layers that make up the light-sensitive material have sensitivity. Any known light sources may be used and they include daylight (sunshine), tungsten lamps, fluorescent lamps, mercury lamps, xenon arc lamps, carbon arc lamps, xenon flash lamps, CRT flying spot, light from a variety of lasers, LED emitted light, and light emitted from fluorescent materials upon excitation by electron beams, X-rays, gamma-rays or alpha-rays.

The exposure time may range from 1 millisecond to 1 second as is usually the case with cameras. Periods shorter than 1 microsecond, such as one ranging from 100 microseconds to 1 microsecond may be employed with CRTs or xenon flash lamps. Exposure longer than 1 second would also be possible. The exposure may be continuous or intermittent.

The silver halide photographic material of the present invention may form an image by any techniques of color development that are known in the art. The color developer used to process this photographic material may contain any of the known aromatic primary amine color developing agents that are extensively used in various color photographic processes. Such developing agents include aminophenolic and p-phenylenediamine derivatives. These compounds are generally used in salt forms, such as hydrochlorides or sulfates, which are stabler than the free state. These compounds are used in concentrations that generally range from about 0.1 to about 30 g, preferably from about 1 g to about 1.5 g per liter of the color developer.

Illustrative aminophenolic developing agents include o-aminophenol, p-aminophenol, 5-amino-2-oxytoluene, 2-amino-3-oxytoluene, and 2-oxy-3-amino-1,4-dimethylbenzene.

Particularly useful primary aromatic amino color developing agents are N,N-dialkyl-p-phenylenediamine compounds wherein the alkyl or phenyl group may have a suitable substituent. Among these compounds, the following are particularly advantageous: N,N'-diethyl-p-phenylenediamine hydrochloride, N-methyl-p-phenylenediamine hydrochloride, N,N'-dimethyl-p-phenylenediamine hydrochloride, 2-amino-5-(N-ethyl-N-dodecylamino)-toluene, N-ethyl-N-β-methanesulfonamidoethyl-3-methyl-4-aminoaniline sulfate, N-ethyl-N-β-hydroxyethylaminoaniline, 4-amino-3-methyl-N,N'-diethylaniline, and 4-amino-N-(2-methoxyethyl)-N-ethyl-3-methylaniline-p-toluene sulfonate.

In addition to these primary aromatic amino color developing agents, the color developer used in the processing of the photographic material of the present invention may contain a variety of additives that are commonly incorporated in color developers and such additives include alkali agents (e.g. sodium hydroxide, sodium carbonate and potassium carbonate), alkali metal sulfites, alkali metal bisulfites, alkali metal thiocyanates, alkali metal halides, benzyl alcohol, water softeners and thickeners. The pH of the color developer is usually at least 7 and most generally ranges from about 10 to about 13.

After color development, the photographic material of the present invention is processed by a solution having the fixing ability. If this solution is a fixing bath, its use is preceded by a bleaching step. The bleaching agent used in the bleaching bath is a metal complex salt of an organic acid. This metal complex salt has the ability not only to oxidize metallic silver (i.e., formed as

5 a result of development) into silver halide but also to ensure complete color formation by a color former. The structure of this metal complex salt is such that an organic acid such as an aminopolycarboxylic acid, oxalic acid or citric acid is coordinated to a metal ion such as iron, cobalt or copper. The organic acids most preferred for use in forming metal complex salts are polycarboxylic acids or aminopolycarboxylic acids. The polycarboxylic acids or aminopolycarboxylic acids may be in the form of alkali metal salts, ammonium salts or water-soluble amine salts.

Typical examples of polycarboxylic acids or aminopolycarboxylic acids are listed below:

- (1) ethylenediaminetetraacetic acid;
- (2) nitrilotriacetic acid;
- (3) iminodiacetic acid;
- (4) ethylenediaminetetraacetic acid disodium salt;
- (5) ethylenediaminetetraacetic acid tetra(trimethylammonium) salt;
- (6) ethylenediaminetetraacetic acid tetrasodium salt; and
- (7) nitrilotriacetic acid sodium salt.

In addition to metal complex salts of these organic acids which are used as bleaching agents, the bleaching bath used in processing the color photographic material of the present invention may contain a variety of additives, and preferred additives are rehalogenating agents such as alkali or ammonium halides (e.g., potassium bromide, sodium bromide, sodium chloride and ammonium bromide), metal salts and chelating agents. Any other additives that are conventionally incorporated in bleaching baths may also be used and they include pH buffers (e.g., borate, oxalate, acetate, carbonate and phosphate salts), alkylamines and polyethylene oxides.

The fixing bath and bleach-fixing bath may also contain one or more pH buffers that are selected from among sulfites (e.g., ammonium sulfite, potassium sulfite, ammonium bisulfite, potassium bisulfite, sodium bisulfite, ammonium metabisulfite, potassium metabisulfite, and sodium metabisulfite), and a variety of acids or salts (e.g., boric acid, borax, sodium hydroxide, potassium hydroxide, sodium carbonate, potassium carbonate, sodium bicarbonate, sodium bisulfite, potassium bicarbonate, acetic acid, sodium acetate and ammonium hydroxide).

If the photographic material of the present invention is processed in a bleach-fixing bath as it is supplied with a blix replenisher, thiosulfates, thiocyanates, sulfites or other salts may be incorporated either in the bleach-fixing bath or in the replenisher that is fed to said blix bath.

In order to increase the activity of the bleach-fixing bath used in processing the photographic material of the present invention, air or oxygen may be blown into a tank containing the bleach-fixing bath or its replenisher. Alternatively, a suitable oxidant such as hydrogen peroxide, bromate or persulfate may be added into the tank.

#### ADVANTAGES OF THE INVENTION

Color photographic materials containing the magenta coupler of the present invention and a magenta dye image stabilizer represented by formula (II) are improved in the fastness of magenta dye images particularly against light, heat and humidity; that is, the discoloration and fading of color against light as well as the occurrence of yellow stain in the background due to light, heat and humidity are satisfactorily prevented.

The advantages of the present invention are hereinunder described in greater detail by reference to working

examples which are given here for illustrative purposes only and are by no means intended as limiting the invention.

## EXAMPLE 1

Gelatin (15.0 mg/100 cm<sup>2</sup>) and comparative magenta coupler (1) (6.0 mg/100 cm<sup>2</sup>) were dispersed in 2,5-di-tert-octylhydroquinone (0.8 mg/100 cm<sup>2</sup>). The dispersion was mixed with a silver chlorobromide emulsion (containing 80 mol% of silver bromide) and the mixture was coated onto a paper support laminated with polyethylene on both surfaces, so as to provide a silver deposit of 3.8 mg/100 cm<sup>2</sup>. The so formed emulsion layer was dried to prepare sample No. 1.

To sample No. 1, a magenta dye image stabilizer in accordance with the invention (PH-13) was added in an amount equimolar to that of the magenta coupler, thereby preparing sample No. 2.

Sample Nos. 3, 6 and 9 were prepared as in the case of sample No. 1 except that comparative magenta coupler (1) was replaced by PC-10, PC-11 and PC-12, three of the triazole type magenta couplers defined in the present invention.

Samples Nos. 4, 7 and 10 were prepared by modifying sample Nos. 3, 6 and 9 with PH-13 added in an amount equimolar to that of the magenta coupler. Sample Nos. 5, 8 and 11 were prepared by modifying sample Nos. 3, 6 and 9 with A-1, another magenta dye image stabilizer within the scope of the invention, added in an amount equimolar to that of the magenta coupler.

Each of the samples thus prepared was exposed through an optical wedge by the conventional method and subsequently processed by the following scheme.

| Steps             | Temperature, °C. | Time             |
|-------------------|------------------|------------------|
| Color development | 33               | 3 min and 30 sec |
| Bleach-fixing     | 33               | 1 min and 30 sec |
| Washing           | 33               | 3 min            |
| Drying            | 50-80            | 2 min            |

35

5

10

15

20

25

30

35

-continued

|                                                                     |          |
|---------------------------------------------------------------------|----------|
| Diethylene glycol                                                   | 10 ml    |
| Potassium carbonate                                                 | 25 g     |
| Sodium bromide                                                      | 0.6 g    |
| Anhydrous sodium sulfite                                            | 2.0 g    |
| Hydroxylamine sulfate                                               | 2.5 g    |
| N-ethyl-N-β-methanesulfonamidoethyl-3-methyl-4-aminoaniline sulfate | 4.5 g    |
| Water to make                                                       | 1,000 ml |
| pH adjusted to 10.2 with NaOH.                                      |          |
| <u>Bleach-fixing bath:</u>                                          |          |
| Ammonium thiosulfate                                                | 120 g    |
| Sodium metabisulfite                                                | 15 g     |
| Anhydrous sodium sulfite                                            | 3 g      |
| EDTA iron (III) ammonium salt                                       | 65 g     |
| Water to make                                                       | 1,000 ml |
| pH adjusted to 6.7-6.8.                                             |          |

Each of the processed samples was placed under illumination in a xenon fadeometer for 8 days so as to examine the light fastness of the dye image and Y staining in the background. Another set of the processed samples were left for 14 days in a hot and humid atmosphere (60° C. × 80% RH) so as to examine the resistance of the dye image to moisture and Y staining in the background. The results are shown in Table 1.

The light fastness and moisture resistance of each sample were evaluated on the following bases.

## Residual dye:

The density of the dye remaining after each of the tests on light fastness and moisture resistance was indicated as a percentage of the initial density (1.0).

## YS:

The density of Y stain before each test was subtracted from the value after testing.

## Discoloration:

The ratio of yellow density to magenta density as measured before testing for an initial density of 1.0 was subtracted from the value after testing. The greater the value obtained, the greater the discoloration from the pure magenta to a yellowish magenta color.

TABLE 1

| Sample No.                   | Coupler                         | Dye image stabilizer | Light fastness   |      |               | Moisture resistance |      |
|------------------------------|---------------------------------|----------------------|------------------|------|---------------|---------------------|------|
|                              |                                 |                      | Residual dye (%) | YS   | Discoloration | Residual dye (%)    | YS   |
| 1 (Comparative)              | Comparative magenta coupler (1) | —                    | 56               | 0.53 | 0.31          | 88                  | 0.59 |
| 2 (Comparative)              | Comparative magenta coupler (1) | PH-13                | 85               | 0.54 | 0.27          | 89                  | 0.60 |
| 3 (Comparative)              | PC-10                           | —                    | 23               | 0.04 | 0.83          | 101                 | 0.07 |
| 4 (Comparative)              | "                               | PH-13                | 75               | 0.10 | 0.79          | 100                 | 0.06 |
| 5 (Sample of the invention)  | "                               | A-1                  | 81               | 0.05 | 0.09          | 101                 | 0.07 |
| 6 (Comparative)              | PC-11                           | —                    | 14               | 0.05 | 0.89          | 100                 | 0.08 |
| 7 (Comparative)              | "                               | PH-13                | 72               | 0.12 | 0.81          | 100                 | 0.07 |
| 8 (sample of the invention)  | "                               | A-1                  | 80               | 0.05 | 0.10          | 99                  | 0.07 |
| 9 (comparative)              | PC-12                           | —                    | 24               | 0.05 | 0.79          | 98                  | 0.07 |
| 10 (comparative)             | "                               | PH-13                | 75               | 0.10 | 0.72          | 100                 | 0.08 |
| 11 (Sample of the invention) | "                               | A-1                  | 82               | 0.06 | 0.07          | 100                 | 0.08 |

The processing solutions used had the following compositions.

65

Color developer:  
Benzyl alcohol

12 ml

Comparative magenta coupler (1)



As is clear from Table 1, Sample Nos. 3, 6 and 9, 15 using the magenta couplers within the scope of the invention, were highly resistant to Y staining as compared with sample No. 1 using the conventional four-equivalent 3-anilino-1,2-pyrazolo-5-one coupler. However, the results of the light fastness test with respect to residual dye and discoloration show that sample Nos. 3, 6 and 9 discolored and faded quite easily upon exposure to light. Sample Nos. 4, 7 and 10 used the magenta couplers of the present invention in combination with PH-13, a conventional magenta dye image stabilizer.

These samples exhibited an appreciable reduction in the fading of dye image resulting from exposure to light, but their resistance to discoloration was not improved at all.

5 Sample Nos. 5, 8 and 11 using magenta couplers and a magenta dye image stabilizer, both in accordance with the present invention, experienced small degrees of discoloration and fading upon exposure to light, heat and moisture, and the Y staining occurring in the background was negligible. These results were certainly unobtainable by sample No. 2 using the conventional four-equivalent 3-anilino-1,2-pyrazolo-5-one magenta coupler and PH-13 (conventional magenta dye image stabilizer).

#### EXAMPLE 2

Sample Nos. 12-35 were prepared as in Example 1 except that the combinations of magenta coupler and magenta dye image stabilizer were changed to those indicated in Table 2. These samples were processed as in Example 1 and subsequently tested for their light-fastness and moisture resistance as in Example 1. The results are shown in Table 2.

TABLE 2

| Sample No.                   | Coupler                         | Dye image stabilizer | Light fastness   |      |               | Moisture resistance |      |
|------------------------------|---------------------------------|----------------------|------------------|------|---------------|---------------------|------|
|                              |                                 |                      | Residual dye (%) | YS   | Discoloration | Residual dye (%)    | YS   |
| 12 (Comparative)             | Comparative magenta coupler (2) | A-1                  | 54               | 0.61 | 0.32          | 87                  | 0.53 |
| 13 (Comparative)             | Comparative magenta coupler (2) | A-2                  | 51               | 0.58 | 0.33          | 85                  | 0.60 |
| 14 (Comparative)             | Comparative magenta coupler (2) | E-2                  | 53               | 0.67 | 0.34          | 83                  | 0.57 |
| 15 (Comparative)             | Comparative magenta coupler (2) | PH-8                 | 82               | 0.51 | 0.27          | 88                  | 0.59 |
| 16 (Comparative)             | Comparative magenta coupler (3) | A-19                 | 56               | 0.63 | 0.37          | 82                  | 0.61 |
| 17 (Comparative)             | Comparative magenta coupler (3) | PH-10                | 83               | 0.54 | 0.27          | 86                  | 0.52 |
| 18 (Comparative)             | PC-15                           | PH-8                 | 72               | 0.13 | 0.87          | 101                 | 0.08 |
| 19 (Comparative)             | "                               | PH-10                | 69               | 0.14 | 0.81          | 100                 | 0.09 |
| 20 (Comparative)             | PC-18                           | PH-8                 | 73               | 0.11 | 0.79          | 98                  | 0.07 |
| 21 (Comparative)             | "                               | PH-10                | 73               | 0.16 | 0.76          | 97                  | 0.09 |
| 22 (Sample of the invention) | PC-15                           | A-1                  | 77               | 0.04 | 0.10          | 100                 | 0.07 |
| 23 (Sample of the invention) | "                               | A-2                  | 78               | 0.03 | 0.09          | 101                 | 0.08 |
| 24 (Sample of the invention) | "                               | A-19                 | 81               | 0.05 | 0.09          | 98                  | 0.09 |
| 25 (Sample of the invention) | "                               | E-2                  | 76               | 0.05 | 0.12          | 102                 | 0.08 |
| 26 (Sample of the invention) | PC-18                           | A-1                  | 81               | 0.04 | 0.08          | 100                 | 0.08 |
| 27 (Sample of the invention) | "                               | A-2                  | 77               | 0.06 | 0.07          | 103                 | 0.07 |
| 28 (Sample of the invention) | "                               | A-19                 | 76               | 0.05 | 0.09          | 100                 | 0.09 |
| 29 (Sample of the invention) | "                               | E-2                  | 81               | 0.04 | 0.08          | 98                  | 0.08 |
| 30 (Sample of the invention) | "                               | B-2                  | 73               | 0.05 | 0.10          | 100                 | 0.08 |
| 31 (Sample of the invention) | "                               | C-4                  | 75               | 0.04 | 0.11          | 101                 | 0.09 |
| 32 (Sample of the invention) | "                               | D-1                  | 70               | 0.05 | 0.10          | 100                 | 0.07 |
| 33 (Sample of the invention) | "                               | H-1                  | 72               | 0.06 | 0.09          | 99                  | 0.09 |
| 34 (Sample of the invention) | "                               | E-3                  | 80               | 0.05 | 0.10          | 101                 | 0.08 |

TABLE 2-continued

| Sample No.                   | Coupler | Dye image stabilizer | Light fastness   |      |               | Moisture resistance |      |
|------------------------------|---------|----------------------|------------------|------|---------------|---------------------|------|
|                              |         |                      | Residual dye (%) | YS   | Discoloration | Residual dye (%)    | YS   |
| 35 (Sample of the invention) | "       | E-4                  | 81               | 0.04 | 0.10          | 100                 | 0.08 |

### Comparative magenta coupler (2)



As Table 2 clearly shows, sample Nos. 12, 13, 14 and 16 using the conventional four-equivalent 3-anilino-1,2-pyrazolo-5-one coupler in combination with magenta dye image stabilizers within the scope of the invention, and sample Nos. 18, 19, 20 and 21 using the combination of magenta couplers falling within the scope of the invention and commonly employed magenta dye image stabilizers were unable to give satisfactory results in all aspects of the light-fastness test and moisture resistance test. The intended results were obtained only when the magenta couplers within the scope of the invention were combined with magenta dye image stabilizers within the scope of the invention. Particularly good results were obtained when magenta dye image stabilizers of formula (XI) or (XII) were used.

### EXAMPLE 3

A paper support laminated with polyethylene on both sides was coated with the following photographic layers in sequence, with the first layer (blue-sensitive silver halide emulsion layer) positioned closest to the support. As a result, sample No. 36 of multi-colored silver halide photographic material was obtained.

This layer was formed by coating 6.8 mg/100 cm<sup>2</sup> of  $\alpha$ -pivaloyl-(2,4-dioxo-1-benzylimidazolidin-3-yl)-2-chloro-5-[ $\gamma$ -(2,4-di-t-amylphenoxy)butylamido]acetanilide (yellow coupler), 3.2 mg/100 cm<sup>2</sup>, in terms of silver, of a blue-sensitive silver chlorobromide emulsion (85 mol% silver bromide), 3.5 mg/100 cm<sup>2</sup> of dioctyl phthalate and 13.5 mg/100 cm<sup>2</sup> of gelatin.

### Second layer: intermediate layer

This layer was formed by coating 0.5 mg/100 cm<sup>2</sup> of 2,5-di-octylhydroquinone, 0.5 mg/100 cm<sup>2</sup> of dinonyl phthalate and 9.0 mg/100 cm<sup>2</sup> of gelatin.

#### Third layer: green-sensitive silver halide emulsion layer

This layer was formed by coating 3.5 mg/100 cm<sup>2</sup> of PC-10 (a magenta coupler included in the scope of the invention), 2.5 mg/100 cm<sup>2</sup>, in terms of silver, of a blue-sensitive silver chlorobromide emulsion (80 mol% silver bromide), 3.0 mg/100 cm<sup>2</sup> of dioctyl phthalate and 12.0 mg/100 cm<sup>2</sup> of gelatin.

#### Fourth layer: intermediate layer

This layer was formed by coating 7.0 mg/100 cm<sup>2</sup> of 2-(2-hydroxy-3-sec-butyl-5-t-butylphenyl)benzotriazole

10 (UV absorber), 6.0 mg/100 cm<sup>2</sup> of dibutyl phthalate, 0.5 mg/100 cm<sup>2</sup> of 2,5-di-t-octylhydroquinone and 12.0 mg/100 cm<sup>2</sup> of gelatin.

### **Fifth layer: red-sensitive silver halide emulsion layer**

This layer was formed by coating 4.2 mg/100 cm<sup>2</sup> of 2-[ $\alpha$ -(2,4-di-t-pentylphenoxy)butanamido]-4,6-dichloro-5-ethylphenol, 3.5 mg/100 cm<sup>2</sup> of tri-2-ethylhexyl phosphate and 11.5 mg/100 cm<sup>2</sup> of gelatin.

### Sixth layer: protective layer

This layer was formed by coating 8.0 mg/100 cm<sup>2</sup> of 20 gelatin.

Sample Nos. 37 to 45 were prepared by modifying sample No. 36 with magenta dye image stabilizers of the present invention that were incorporated in the 3rd layer in the amounts indicated in Table 3. Sample Nos. 36 to 45 were processed as in Example 1 and subjected to a light-fastness test under illumination in a xenon fedeometer for 15 days. The test results are shown in Table 3.

TABLE 3

| Sample No.                                     | Dye image stabilizer | Amount of stabilizer (mol %/coupler) | Residual magenta dye (%) |
|------------------------------------------------|----------------------|--------------------------------------|--------------------------|
| 36 (Comparative)<br>(Samples of the invention) | —                    | —                                    | 17                       |
| 37                                             | A-2                  | 50                                   | 58                       |
| 38                                             | "                    | 100                                  | 67                       |
| 39                                             | "                    | 150                                  | 85                       |
| 40                                             | A-19                 | 50                                   | 55                       |
| 41                                             | "                    | 100                                  | 73                       |
| 42                                             | "                    | 150                                  | 88                       |
| 43                                             | E-2                  | 50                                   | 57                       |
| 44                                             | "                    | 100                                  | 69                       |
| 45                                             | "                    | 150                                  | 84                       |

The data in Table 3 show that the magenta dye image stabilizers in accordance with the present invention are effective in stabilizing the dye image formed by the triazole type magenta coupler of the present invention and that this effectiveness is increased as the amounts in which these stabilizers are incorporated is increased. Sample Nos. 37 to 45 experienced a very small amount of discoloration in the magenta image as a result of exposure to light. Furthermore, these samples of the present invention suffered an extremely small degree of fading in the magenta dye. Therefore, they struck a good color balance between yellow, cyan and magenta couplers and displayed a highly satisfactory color reproduction.

**EXAMPLE 4**

Gelatin (15.0 mg/100 cm<sup>2</sup>) and comparative magenta coupler (1) (6.0 mg/100 cm<sup>2</sup>) were dispersed in dibutylphthalate (0.8 mg/100 cm<sup>2</sup>) together with 2,5-di-tert-octylhydroquinone (0.8 mg/100 cm<sup>2</sup>). The dispersion was mixed with a silver chlorobromide emulsion (containing 80 mol% of silver bromide) and the mixture was coated onto a paper support laminated with polyethylene on both surfaces, so as to provide a silver deposit of

3.8 mg/100 cm<sup>2</sup>. The so formed emulsion layer was dried to prepare sample No. 46.

To sample No. 46, a magenta dye image stabilizer in accordance with the invention (PH-13) was added in an amount equimolar to that of the magenta coupler, 5 thereby preparing sample No. 47.

Sample Nos. 48, 51 and 54 were prepared as in the case of sample No. 46 except that comparative magenta coupler (1) was replaced by PC-39, PC-41 and PC-130, three of the magenta couplers defined in the present 10 invention.

Sample Nos. 49, 52 and 55 were prepared by modifying sample Nos. 48, 51 and 54 with PH-13 added in an amount equimolar to that of the magenta coupler. Sample Nos. 50, 53 and 56 were prepared by modifying 15 sample Nos. 48, 51 and 54 with A-1 in place of PH-13, another magenta dye image stabilizer within the scope of the invention, added in an amount equimolar to that of the magenta coupler.

#### Comparative magenta coupler (1)



Each of the samples thus prepared was exposed through an optical wedge by the conventional method and subsequently processed by the following scheme.

| Step              | Temperature, °C. | Time             |
|-------------------|------------------|------------------|
| Color development | 33               | 3 min and 30 sec |
| Bleach-fixing     | 33               | 1 min and 30 sec |

40

35 The density of Y stain before each test was subtracted from the value after testing.

#### Discoloration:

The ratio of yellow density to magenta density as measured before testing for an initial density of 1.0 was subtracted from the value after testing. The greater the value obtained, the greater the discoloration from the pure magenta to a yellowish magenta color.

TABLE 4

| Sample No.                   | Coupler                         | Dye image stabilizer | Light fastness   |      |               | Moisture resistance |      |
|------------------------------|---------------------------------|----------------------|------------------|------|---------------|---------------------|------|
|                              |                                 |                      | Residual dye (%) | YS   | Discoloration | Residual dye (%)    | YS   |
| 46 (Comparative)             | Comparative magenta coupler (1) | —                    | 50               | 0.54 | 0.34          | 88                  | 0.53 |
| 47 (Comparative)             | Comparative magenta coupler (1) | PH-13                | 79               | 0.51 | 0.27          | 89                  | 0.56 |
| 48 (Comparative)             | PC-39                           | —                    | 22               | 0.06 | 0.78          | 101                 | 0.07 |
| 49 (Comparative)             | "                               | PH-13                | 70               | 0.10 | 0.74          | 102                 | 0.08 |
| 50 (Sample of the invention) | "                               | A-1                  | 77               | 0.05 | 0.14          | 101                 | 0.06 |
| 51 (Comparative)             | PC-41                           | —                    | 23               | 0.06 | 0.74          | 102                 | 0.06 |
| 52 (Comparative)             | "                               | PH-13                | 69               | 0.07 | 0.70          | 100                 | 0.07 |
| 53 (Sample of the invention) | "                               | A-1                  | 76               | 0.07 | 0.14          | 98                  | 0.08 |
| 54 (Comparative)             | PC-130                          | —                    | 15               | 0.08 | 0.88          | 100                 | 0.09 |
| 55 (Comparative)             | "                               | PH-13                | 63               | 0.11 | 0.80          | 97                  | 0.10 |
| 56 (Sample of the invention) | "                               | A-1                  | 69               | 0.09 | 0.17          | 101                 | 0.10 |

|         |       |        |
|---------|-------|--------|
| Washing | 33    | 3 min  |
| Drying  | 50-80 | 2 min. |

65

The processing solutions used had the following compositions.

| Color developer:                                                    |          |
|---------------------------------------------------------------------|----------|
| Benzyl alcohol                                                      | 12 ml    |
| Diethylene glycol                                                   | 10 ml    |
| Potassium carbonate                                                 | 25 g     |
| Sodium bromide                                                      | 0.6 g    |
| Anhydrous sodium sulfite                                            | 2.0 g    |
| Hydroxylamine sulfate                                               | 2.5 g    |
| N-ethyl-N-β-methanesulfonamidoethyl-3-methyl-4-aminoaniline sulfate | 4.5 g    |
| Water to make                                                       | 1,000 ml |
| pH adjusted to 10.2 with NaOH                                       |          |
| Bleach-fixing bath:                                                 |          |
| Ammonium thiosulfate                                                | 120 g    |
| Sodium metabisulfite                                                | 15 g     |
| Anhydrous sodium sulfite                                            | 3 g      |
| EDTA iron (III) ammonium salt                                       | 65 g     |
| Water to make                                                       | 1,000 ml |
| pH adjusted to 6.7-6.8.                                             |          |

Each of the processed samples was placed under 20 illumination in a xenon fadeometer for 8 days so as to examine the light fastness of the dye image and Y staining in the background. Another set of the processed samples were left for 14 days in a hot and humid atmosphere (60° C. × 80% RH) so as to examine the resistance 25 of the dye image to moisture and Y staining in the background. The results are shown in Table 1.

The light fastness and moisture resistance of each sample were evaluated on the following bases.

#### Residual dye:

30 The density of the dye remaining after each of the tests on light fastness and moisture resistance was indicated as a percentage of the initial density (1.0).

#### YS:

35 The density of Y stain before each test was subtracted from the value after testing.

#### Discoloration:

The ratio of yellow density to magenta density as measured before testing for an initial density of 1.0 was subtracted from the value after testing. The greater the value obtained, the greater the discoloration from the pure magenta to a yellowish magenta color.

TABLE 4

As is clear from Table 4, sample Nos. 48, 51 and 54, using the magenta couplers within the scope of the invention, were highly resistant to Y staining as compared with sample No. 46 using the conventional four-equivalent 3-anilino-5-pyrazolone coupler. However,

the results of the light fastness test with respect to residual dye and discoloration show that sample Nos. 48, 51 and 54 discolored and faded quite easily upon exposure to light. Sample Nos. 49, 52 and 53 used the magenta couplers of the present invention in combination with PH-13, a conventional magenta dye image stabilizer. These samples exhibited an appreciable reduction in the fading of dye image resulting from exposure to light, but their resistance to discoloration was not improved at all.

Sample Nos. 50, 53 and 56 using magenta couplers and a magenta dye image stabilizer, both in accordance with the present invention, experienced small degrees of discoloration and fading upon exposure to light, heat and moisture, and the Y staining occurring in the background was negligible. These results were certainly unobtainable by sample No. 47 using the conventional four-equivalent 3-anilino-5-pyrazolone coupler and PH-13 (conventional magenta dye image stabilizer).

**EXAMPLE 5**

Sample Nos. 57-72 were prepared as in Example 4 except that the combinations of magenta coupler and magenta dye image stabilizer were changed to those indicated in Table 5. These samples were processed as in Example 4 and subsequently tested for their lightfastness and moisture resistance as in Example 4. The results are shown in Table 5.

TABLE 5



15 (In Table 5, A-2 and PH compounds were used in a molar ratio of 2:1 for sample Nos. 70, 71 and 72, and the total amount of dye image stabilizers was the same amount of mole as those used for other samples.)

amount of mole as those used for other samples.)

As Table 5 clearly shows, sample Nos. 57 and 58 using the conventional four-equivalent 3-anilino-5-pyrazolone coupler in combination with magenta dye image stabilizers within the scope of the invention, and sample Nos. 61, 62, 63 and 64 using the combination of magenta couplers falling within the scope of the invention and commonly employed magenta dye image stabilizers were unable to give satisfactory results in all aspects of the light-fastness test and moisture resistance test. The intended results were obtained only when the

| Sample No.                   | Coupler                         | Dye image stabilizer | Light fastness   |      |               | Moisture resistance |      |
|------------------------------|---------------------------------|----------------------|------------------|------|---------------|---------------------|------|
|                              |                                 |                      | Residual dye (%) | YS   | Discoloration | Residual dye (%)    | YS   |
| 57 (Comparative)             | Comparative magenta coupler (2) | A-2                  | 46               | 0.57 | 0.36          | 87                  | 0.51 |
| 58 (Comparative)             | Comparative magenta coupler (2) | D-2                  | 44               | 0.52 | 0.32          | 89                  | 0.54 |
| 59 (Comparative)             | Comparative magenta coupler (2) | PH-8                 | 70               | 0.51 | 0.30          | 88                  | 0.54 |
| 60 (Comparative)             | Comparative magenta coupler (2) | PH-10                | 71               | 0.55 | 0.29          | 86                  | 0.50 |
| 61 (Comparative)             | PC-52                           | PH-8                 | 63               | 0.13 | 0.88          | 100                 | 0.09 |
| 62 (Comparative)             | "                               | PH-10                | 65               | 0.14 | 0.85          | 98                  | 0.10 |
| 63 (Comparative)             | PC-90                           | PH-8                 | 67               | 0.16 | 0.83          | 100                 | 0.10 |
| 64 (Comparative)             | "                               | PH-10                | 68               | 0.15 | 0.81          | 97                  | 0.11 |
| 65 (Sample of the invention) | PC-52                           | A-25                 | 74               | 0.07 | 0.13          | 101                 | 0.08 |
| 66 (Sample of the invention) | "                               | D-2                  | 68               | 0.06 | 0.14          | 99                  | 0.09 |
| 67 (Sample of the invention) | PC-90                           | A-2                  | 74               | 0.05 | 0.14          | 98                  | 0.07 |
| 68 (Sample of the invention) | "                               | D-2                  | 67               | 0.05 | 0.14          | 98                  | 0.09 |
| 69 (Sample of the invention) | "                               | E-3                  | 72               | 0.07 | 0.10          | 99                  | 0.10 |
| 70 (Sample of the invention) | "                               | A-2<br>PH-8          | 78               | 0.08 | 0.20          | 101                 | 0.09 |
| 71 (Sample of the invention) | "                               | A-2<br>PH-10         | 81               | 0.10 | 0.20          | 100                 | 0.10 |
| 72 (Sample of the invention) | "                               | A-2<br>PH-13         | 81               | 0.11 | 0.19          | 100                 | 0.10 |

magenta couplers within the scope of the invention were combined with magenta dye image stabilizers within the scope of the invention.

65 In sample Nos. 70, 71 and 72 using the magenta couplers within the scope of the invention in combination with the magenta dye image stabilizers within the scope of the invention and the conventional dye image stabi-





wherein

R<sub>1</sub> and R<sub>8</sub> each represents a hydrogen atom or a substituent; and

X represents a hydrogen atom or a substituent capable of leaving upon reaction with the oxidized product of a color developing agent.

3. A silver halide color photographic material according to claim 1, wherein the substituent represented by R in said formula (I) is one represented by the following formula:



wherein R<sub>9</sub>, R<sub>10</sub> and R<sub>11</sub> each represents a hydrogen atom, a halogen atom, an alkyl group, a cycloalkyl group, an alkenyl group, a cycloalkenyl group, an alkynyl group, an aryl group, a heterocyclic group, an acyl group, a sulfonyl group, a sulfinyl group, a phosphonyl group, a carbamoyl group, a sulfamoyl group, a cyano group, a spiro-compound residue, a bridged hydrocarbon compound residue, an alkoxy group, an aryloxy group, a heterocyclicoxy group, a siloxy group, an acyloxy group, a carbamoyloxy group, an amino group, an acylamino group, a sulfonamide group, an imido group, a ureido group, a sulfamoylamino group, an alkoxy carbonylamino group, an aryloxycarbonylamino group, an alkoxy carbonyl group, an aryloxycarbonyl group, an alkylthio group; an arylthio group or a heterocyclicthio group, provided that at least two of R<sub>9</sub>, R<sub>10</sub> and R<sub>11</sub> are not hydrogen atoms.

4. A silver halide color photographic material according to claim 1, wherein the aliphatic group repre-

sented by R<sub>1</sub> in said formula (II) is a saturated alkyl group or an unsaturated alkyl group.

5. A silver halide color photographic material according to claim 1, wherein the cycloalkyl group represented by R<sub>1</sub> in said formula (II) is 5-to-7-membered ring.

6. A silver halide color photographic material according to claim 1, wherein said compound represented by formula (II) is incorporated in an amount of 5 to 300 mol% with respect to said magenta color image-forming coupler represented by formula (I).

7. A silver halide color photographic material according to claim 1, wherein said magenta color image-forming coupler represented by formula (I) is one represented by the following formula (IX):



wherein

25 R<sub>1</sub> represents a hydrogen atom or a substituent; X represents a hydrogen atom or a substituent capable of leaving upon reaction with the oxidized product of a color developing agent; and Z<sub>1</sub> represents the group of nonmetallic atoms necessary for forming a nitrogen-containing heterocyclic ring, provided that the ring to be formed by said Z<sub>1</sub> may have a substituent.

30 8. A silver halide color photographic material according to claim 1, wherein said magenta color image-forming coupler is one represented by the above-mentioned formula (III).

35 9. A silver halide color photographic material according to claim 2, wherein the substituent capable of leaving upon reaction with the oxidized product of a color developing agent represented by X in said formula (III) represents a halogen atom, an alkoxy group, an aryloxy group, an acyloxy group, a 5- or 6-membered heterocyclicoxy group, an alkylthio group, a 5- or 6-membered heterocyclicthio group or



45 50 (wherein A<sub>1</sub> and A<sub>2</sub> which may be the same or different each represents a hydrogen atom, an alkyl group, an aryl group, a heterocyclic group, an acyl group, a sulfonyl group, a carbamoyl group, a sulfamoyl group, an alkoxycarbonyl group or an aryloxycarbonyl group, provided that both of A<sub>1</sub> and A<sub>2</sub> are not hydrogen atoms at the same time, and A<sub>1</sub> and A<sub>2</sub> may cooperate to form a 5- or 6-membered ring taken together with the nitrogen atom).

60 65 10. A silver halide color photographic material according to claim 2, wherein R<sub>1</sub> and R<sub>2</sub> of said formula (III) each represents a hydrogen atom, an alkyl group, an aryl group, a heterocyclic group, an acylamino group, an anilino group, an alkoxy carbonyl group or an alkylthio group.

\* \* \* \* \*